

Patented Dec. 23, 1924.

1,520,380

# UNITED STATES PATENT OFFICE.

GUSTAV WETTER, OF WEESEN, SWITZERLAND.

## WRITING BOARD OR SLATE AND METHOD OF MAKING SAME.

No Drawing.

Application filed August 29, 1921. Serial No. 496,656.

(GRANTED UNDER THE PROVISIONS OF THE ACT OF MARCH 3, 1921, 41 STAT. L., 1313.)

*To all whom it may concern:*

Be it known that I, GUSTAV WETTER, a citizen of the Republic of Switzerland, residing at Weesen, Switzerland, have invented certain new and useful Improvements in Writing Boards or Slates and Methods of Making Same (for which I have filed applications in Switzerland August 26, 1920, and in Germany on September 7th, 1920),

10 of which the following is a specification.

This invention relates to improvements in a method for making writing boards and slates. It has already been proposed in preparing the writing surface of slates and the like, on which the writing must be easily obliterated, to utilize water-glass and earthy colors with certain additions for instance of silicate of magnesia or of silicic acid and pulverulent carbonate of lime, which mixture is applied as a covering layer to a base part. Writing surfaces of this kind have not proved successful as it has been found extremely difficult to apply a uniform covering layer of such materials and further this layer becomes hard, cracked and blisters.

The object of the present invention is to overcome the above mentioned disadvantages and to provide for a durable writing surface that responds to all the requirements. According to the invention the covering layer applied to a base part consists of water-glass and zinc-white to which a further covering layer of a solution of water-glass is applied. To the first layer consisting of water-glass and zinc-white a small addition of a colouring matter may be made in order to produce a writing surface of a desired colour.

40 As base cardboard, paper, wood, asbestos cement, slate, steel plate or other materials

may be used. Writing on the surface prepared according to the invention can be effected with pencil, coloured crayon or the like as well as with water colours or an ink 45 that is free of acids. The writing or drawing may easily and completely be obliterated by means of a sponge or the like.

The slate itself may be of any shape. It may also be provided with a frame. 50

I claim:

1. A process for preparing writing surfaces on slates, boards and the like, consisting in applying a cover layer of water-glass and zinc-white to a surface of a base, 55 and in applying a layer of a water-glass solution to said covering layer.

2. A process for preparing writing surfaces on slates, boards and the like, consisting in applying a covering layer of water-glass and zinc-white with an addition of a colouring matter to a surface of a base, and in applying a layer of a water-glass solution to said covering layer. 60

3. A slate or board for writing purposes, 65 comprising a base adapted to form at least one writing surface, a covering layer consisting of water-glass and zinc-white applied to said writing surface, and a layer consisting solely of water-glass applied to said covering layer. 70

4. A slate or board for writing purposes, comprising a base adapted to form at least one writing surface, a covering layer consisting of water-glass and zinc-white with 75 an addition of colouring matter applied to said writing surface, and a layer consisting solely of water-glass applied to said covering layer.

In testimony whereof I affix my signature. 80

GUST WETTER.